

## UNITED STATES PATENT OFFICE

HAROLD ROBERT RAFTON, OF LAWRENCE, MASSACHUSETTS, ASSIGNOR TO RAFFOLD PROCESS CORPORATION, A CORPORATION OF MASSACHUSETTS

## PAPER PRODUCT AND METHOD OF MAKING THE SAME

No Drawing.

Application filed September 5, 1928. Serial No. 304,170.

This invention relates to the manufacture of paper and more particularly to an improved sized paper containing a carbonate filler and a method of making the same.

5 The principal object of this invention is to provide a process of sizing paper made with a carbonate filler wherein paraffin is employed as the sizing agent, the paraffin being employed in the form of a substantially 10 nonbreakable emulsion, the disperse phase of such emulsion being concentrated by the mutual precipitation or flocculation of two suitable precipitating agents in the presence of the emulsion.

15 An important object of this invention is to provide an economical and efficient process of making an improved sized paper made with a carbonate filler wherein the disperse phase of a substantially nonbreakable paraffin emulsion is concentrated by the mutual 20 precipitation or flocculation of sodium resinate and alum.

Another object of this invention is to provide a simple and efficient process of making 25 an improved sized paper made with a carbonate filler wherein a substantially non-breakable paraffin emulsion is employed as a sizing agent and wherein two mutual precipitating agents are employed for concentrat- 30 ing the disperse phase of the paraffin emulsion, the sizing effect of the sizing agent which is wholly or in part deteriorated by the action of the carbonate filler employed being restored by the subsequent addition of a suitable 35 sizing restoring agent.

A further object of this invention is to provide a paper making process of the above referred to character wherein sodium resinate and alum are employed for concentrating the 40 disperse phase of the paraffin emulsion employed and wherein alum is employed as a sizing restoring agent.

Other objects and advantages of this invention will become apparent during the 45 course of the following description.

In my copending application Serial No. 304,169 filed Sept. 5, 1928, I have described a method of using a substantially nonbreakable paraffin emulsion as a sizing agent in the 50 manufacture of paper wherein the mutual flocculation of two suitable reacting agents such as sodium resinate and alum is employed to concentrate the disperse phase of such emulsion and bring it into association with the fibre employed. The method of sizing 55 described therein refers to paper made without filler or with ordinary fillers such, for example, as clay or talc. The present invention relates to the similar use of a substantially nonbreakable paraffin emulsion as 60 sizing for papers which contain carbonate fillers. In this case it is found that the carbonate fillers cause deterioration of the sizing effect when used in the place of ordinary fillers such as clay for example, and the method 65 of circumventing this deterioration of sizing by the carbonate filler by the expedient of restoring the sizing with a suitable agent after the deterioration of the sizing has taken place is dealt with herein. An analogous 70 method is disclosed in my copending application Serial No. 304,168 filed Sept. 5, 1928, for use when rosin size is the sizing agent employed.

As will be apparent to those skilled in the art, it is substantially the universal practice in sizing paper to mix with suitable fibrous materials and filler, if such is to be employed, sodium resinate, and to precipitate the sodium resinate with alum in the presence of 80 the fibre. While the order of addition of these ingredients may be and is varied in different processes it has been generally accepted that the addition of both sodium resinate and alum, or equivalent thereof, is necessary 85 for imparting suitable sizing to the finished paper. As is well known, the so-called sodium resinate employed in paper making processes is not always this exact compound nor, when this compound is used, is it necessarily chemically pure, it generally containing varying amounts of uncombined rosin and sometimes uncombined alkali. However, where this term is employed herein it is to be understood that the term includes 90 any material produced by the action of alkali, generally in aqueous solution, on rosin, or on natural or synthetic resin acid or acids, regardless of the exact composition of the prod-

100

uct or the varying composition which different samples of the product may possess.

Sized paper made substantially in accordance with the general method outlined above is not suitable for many purposes and various other types of papers are employed in numerous arts. For example, it has been proposed heretofore to make a water resistant paper by adding to suitable fibre a combination of sodium resinate and a breakable paraffin emulsion, ordinarily a saponaceous emulsion, and to precipitate the paraffin in connection with the rosin on the fibrous material by the use of alum. Paper of this class is commonly called "paraffined paper".

While paraffined papers are suitable for many uses the use of such papers is not general. For example, these papers generally have a paraffin finish which makes them substantially waterproof and are ordinarily translucent or substantially transparent. Hence such papers are not suitable for use as book, magazine, writing or printing papers.

Moreover the use of emulsions particularly of the class referred to above which are employed in making paraffined papers is attended with numerous serious disadvantages as hereinafter more particularly set forth.

As is well known an emulsion of paraffin is a suspension of microscopically minute particles of paraffin in a liquid, ordinarily aqueous or miscible with water, containing an emulsifying agent, i. e., a material or materials which tend to prevent the coalescence of the individual particles of paraffin. The most widely accepted work relating to emulsions points to the fact that there is actually a layer or film of the emulsifying agent one or more molecules in thickness surrounding each particle of emulsified material, which in the case of paraffin is called herein the disperse phase of the emulsion. This film or layer however in certain cases may be of very much greater thickness, for instance in the case where an insoluble emulsifying agent is used. The individual particles of the disperse phase of an emulsion act very differently from the same material in comminuted form in an aqueous medium in which no emulsifying agent is present. In such case the individual particles are not prevented from contacting with each other and in fact the particles do touch and eventually coalesce to form relatively massive lumps of the material. The same material in emulsified form however does not have these characteristics and the individual particles of the disperse phase, such as paraffin, for example, are prevented from touching one another with the result that there is no tendency for the particles to coalesce and form lumps. Although particles in unemulsified condition exhibit different characteristics from similar particles in emulsified condition it is to be point-

ed out that different emulsions differ in several respects but particularly do they differ with regard to their stability. For example, many and undoubtedly the great majority of emulsions tend to resolve or break in the well known manner. It is this characteristic that has led chiefly to the disadvantages surrounding the use of emulsions in paper making processes as heretofore employed. For example, certain emulsions commonly employed for use in paper making such for example as paraffin emulsions are broken by the addition of alum thereto. Moreover, such emulsions can usually be broken by acids and also to some extent by soluble salts such as those which occur in hard water or incompletely washed fibrous materials. This breaking of emulsions such as a paraffin emulsion is accompanied by the rise of the individual particles such as paraffin which are released from the emulsified form, to the surface of the liquid with consequent tendency toward agglomeration and formation of relatively large particles.

When breakable emulsions of the character referred to have been employed heretofore in paper making processes the paraffin has been precipitated in individual particles usually by alum on the fibre while the fibre was in aqueous suspension. In some cases sodium resinate has been employed in connection with such breakable emulsions and the mixture of the sodium resinate and paraffin emulsion has been mutually precipitated on the fibre by means of alum. Of course, in this case as well as in the case where no sodium resinate was employed the paraffin was deposited in individual particles, but in this instance it was commingled with the alum-sodium resinate precipitate. An important factor in each of these cases resides in the direct contact of the finely divided paraffin with the fibre by the direct deposition of the particles out of the emulsified state on to the fibre. These minute individual particles of paraffin are normally nonadhesive but there is a tendency under the conditions of agitation obtaining in the paper making process for some of the particles to become detached from the fibre, which particles may be aggregated by pressure or otherwise so that relatively coarse flakes or lumps of paraffin are formed and exist at the wet end of the paper making machine. These flakes or lumps often cause very serious trouble particularly in the screens, in the web-forming device of the paper machine, and also in various parts of the machine clothing and the press rolls.

It has also been proposed heretofore to make waterproof paper such as roofing paper by mixing an emulsion of asphalt or the like, preferably containing clay as an emulsifying agent, with suitable fibre and running this mix off on a paper machine. These emul-

sions, which are relatively coarse, are retained in the felted sheet by mere mechanical filtration, the proportion of the emulsion used being sufficiently great (sometimes equal to 5 or greater than the amount of fibre present) to insure the retention of a sufficient amount of asphalt in the finished sheet. A modification of this process uses a fixing agent to attach the asphalt to the fibres. Of course, 10 apart from other reasons, because of their color the employment of asphalt or bituminous emulsions is not feasible in making high grade book, magazine, writing or printing paper and the like. Moreover emulsions 15 made with paraffin wherein solid emulsifying agents such as clay are employed have been found to be disadvantageous for the reason inter alia that when such emulsions are employed in small quantities in a sheet such as 20 might be expected to be sufficient to produce a sized paper, the particle size of the paraffin is usually sufficiently large to cause waterproofing to occur in definite spots which are surrounded by areas that are substantially 25 unsized, the finished product thereby resulting in a sheet having a combination of waterproof areas and unsized or only partially sized areas. Moreover emulsions made with insoluble emulsifying agents have certain 30 breakable characteristics as described below and have thus a tendency toward being broken during the paper making process with consequent deposition of paraffin or like material on various parts of the paper making 35 machine and machine clothing.

For instance, some emulsions made with insoluble emulsifying agents have a tendency to be unstable at extreme dilutions. Such emulsions also may be sensitive to pressure, 40 and also are known to be sensitive to the mechanical agencies employed in the paper making process such for example as the beater and the Jordan. Of course in these agencies there tends to be a contacting at high 45 speed between two metal surfaces, and as is natural, this influence will tend to break down the insoluble particle film surrounding the individual particles of emulsified material, and consequently numerous particles of 50 the disperse phase having their protective coating ruptured or removed will tend to coalesce and produce thereby larger or smaller lumps of unemulsified material which will cause trouble in the subsequent machining 55 of the stock. It is therefore apparent that emulsions made with an insoluble emulsifying agent are not sufficiently completely resistant to the mechanical instrumentalities met with in the paper making process and 60 thus they cannot be considered as substantially nonbreakable emulsions.

In my copending application for "Improvements in paper products and methods of making the same", Serial Number 262,030, filed March 15th, 1928, I have described a

method of making a sized carbonate filled paper wherein a paraffin emulsion is employed. In that application I have pointed out the necessity of obtaining as stable an emulsion as feasible, indicating the particular necessity for this where hard water is to be used and/or where the fibrous constituents have not been washed sufficiently to remove such soluble materials as may have a tendency to break the emulsion. Furthermore in that application I have disclosed the mutual flocculation of paraffin emulsions and carbonate fillers to give a unique carbonate filler paraffin complex.

Whereas the method I describe in the above referred to application is satisfactory in some cases, I have found that owing to the difficulty of preventing the premature breaking of the emulsions used it was desirable to find an emulsion which would be substantially nonbreakable under the conditions obtaining in paper making practice up to the point of addition of the carbonate filler. I have found such an emulsion and have also found that such a stable emulsion is not only stable to ordinary paper making procedure, but also is not mutually flocculated with carbonate filler as are the emulsions set out in my application Serial No. 262,030, mentioned above. Hence other means must be employed for permanently associating the emulsion with the paper mix, as will be described in detail below.

My process consists broadly in adding to fibrous material, sodium resinate in a sufficient amount as indicated below and an emulsion of paraffin substantially nonbreakable by any of the chemical or mechanical agencies ordinarily employed in the paper making process in the concentrations or intensities in which they are normally used. Preferably after these are thoroughly mixed I then add alum, then carbonate filler. Prior to the addition of the carbonate filler, if a portion of the mix is withdrawn and made into a sheet in the laboratory, it will be found to be sized, but after the addition of the carbonate filler the mix gradually suffers a deterioration in sizing, although by the time the paper machine is reached there may still be some degree of sizing remaining in the stock in certain cases. However, I have discovered, that the sizing may be restored by the addition of a subsequent quantity of suitable material added preferably at a point in the paper making process where there is opportunity for only a minimum amount of contact of the ingredients of the mix and also only a minimum time of contact. Such a point is at or subsequent to the dilution of the stock in preparation for its delivery to the web-forming end of the paper machine.

The amount of sodium resinate I may use is that amount which by itself when precipitated with alum, and restored with a subse-

quent quantity of alum, in accordance with my copending application Serial No. 304,168 filed Sept. 5, 1928, would not be sufficient to size the paper, but would produce a substantially unsized paper. Thus the precipitate produced by sodium resinate and alum and then subsequently restored does not in this case act as a sizing agent but as a concentrating agent in the manner described below. Of course, I may, if I desire, use a greater quantity of sodium resinate, but it is to be pointed out that it is possible to secure satisfactory sizing by my process where there is not enough sodium resinate used to impart sizing of itself.

As stated above, I have discovered that the use of emulsions which are substantially stable under normal paper making practice wholly avoids the numerous disadvantages commonly encountered in prior processes involving the use of breakable emulsions. However, it will be apparent that the mere use of substantially nonbreakable emulsions does not alone produce the desired results since unless suitable means are provided for effecting the association of such emulsions with the fibrous material they would merely pass off with the effluent waters and not remain associated with the fibre as desired.

I have discovered that substantially nonbreakable emulsions can be brought into the desired association with fibres and held in such association up to the desired point substantially without breaking the emulsions by concentrating the disperse phase of the emulsions by means of two mutually flocculating or precipitating materials, such for example as sodium resinate and alum. This concentration of the disperse phase in the concentrating precipitate however does not break the emulsion.

The fact that treatment in the manner suggested merely concentrates the disperse phase of the emulsion and does not break the emulsion is clearly shown by the following experiment: If a relatively dilute solution of sodium resinate is added to a breakable paraffin emulsion, such as saponaceous paraffin emulsion, and alum is then added in an amount sufficient to completely flocculate both the sodium resinate and the paraffin emulsion, there will result a precipitate and a clear residual liquid. The precipitate will consist of an alum-sodium resinate precipitate and also of an alum-soap precipitate (that is, the soap which is used as the emulsifying agent for the paraffin), and also individual particles of free paraffin released from the emulsified condition. Now if some chemical is added which completely dissolves these alum-sodium resinate and alum-soap compounds, (and which has been found at the concentration used and within the time required for the experiment will not of itself break the paraffin emulsion in question) such

for example as sodium hydroxide, that part of the flocculent precipitate due to the resinate and soap precipitates disappears, and the paraffin which remains undissolved rises to the surface in more or less agglomerated form.

On the other hand, if a substantially non-breakable emulsion of the character herein-after described is similarly mixed with a dilute solution of sodium resinate, and sufficient alum added to completely flocculate the same, it will be found that the precipitate separates, leaving a clear residual liquid. Up to this point the result appears to be exactly the same as in the previous experiment.

However, when sodium hydroxide is added in the manner suggested as above, in an amount sufficient to dissolve the alum-sodium resinate compound, the entire solution becomes milky, no paraffin floats to the surface, and the paraffin emulsion is thus "deconcentrated", i. e., restored to its original condition substantially unbroken. A microscopic examination of the milky liquid shows that the paraffin particles are present in the emulsified condition substantially the same as they were before they were concentrated by the precipitation of the alum-sodium resinate compound. It is apparent, therefore, that the action of the mutually flocculating materials in what appears to be the breaking of this emulsion is in no sense a breaking, but is an instance of the unique concentration of the disperse phase of a substantially non-breakable emulsion without the breaking of such emulsion. This concentration of the disperse phase is substantially completely reversible, i. e., the disperse phase can be deconcentrated or diluted by dissolving the precipitate of the mutually flocculating materials.

In other words in the concentrating precipitate, in this instance the alum-sodium resinate compound, the paraffin of a substantially nonbreakable emulsion does not exist as deposited particles released from emulsified form, and when the reaction is carried out in the presence of fibre the paraffin is not deposited jointly with the alum-sodium resinate precipitate upon the fibre, and does not therefore cause the difficulties experienced in the paper making process, as is the case when breakable emulsions are broken with alum, either alone or in the presence of alum-sodium resinate precipitate in the paper making process.

Moreover when the disperse phase of a substantially nonbreakable paraffin emulsion, concentrated in an alum-sodium resinate precipitate on fibre, is subjected to the beating and jordaning operations in regular paper-making practice, although of course the concentrating precipitate may be mechanically subdivided by these agencies, there is no evidence that any paraffin has been released from

the emulsified condition, the concentrated disperse phase thus being apparently nonbreakable by the mechanical agencies to which it is subjected in the papermaking operation.

5 The alum-sodium resinate precipitate in the present instance, therefore, merely serves as a means for concentrating the disperse phase of an emulsion without breaking the emulsion, the disperse phase in the meantime 10 being maintained in emulsified condition, and substantially nonbreakable by mechanical means. This concentration of the disperse phase appears to produce a complex which experiments indicate to be an intermediate 15 between a true emulsion and a resolved or broken emulsion. For example, the complex can be temporarily dispersed by mechanical means as indicated above but not diluted in the true sense as in the case of true 20 emulsions. However, the complex can in a sense be diluted by dissolving the mutually flocculating agents therein and reconverting to a true emulsion. Thus while it is clear that the complex is not a true emulsion it is 25 on the other hand, not a resolved emulsion. For example, the paraffin is not present in the concentrate as individual unitary deposited particles of paraffin, but rather in emulsified form, each particle being surrounded by a 30 layer or film of emulsifying agent which prevents the individual particles from having contact not only with other particles of paraffin, but also from having contact with either the alum-sodium resinate precipitate, or the 35 fibres, or other constituents of the fibrous mix. The existence of the paraffin in emulsified form is thus continued throughout the entire wet end of the paper making process. It is associated with the solids in the paper mix 40 but is not deposited as paraffin thereon, and thus, as heretofore stated, completely eliminates the difficulties which are present when emulsions are broken with alum, alone or in conjunction with sodium resinate, or by 45 mechanical agencies, in the paper making process. This is a very great advance in the art of sizing paper with paraffin emulsions as will be readily appreciated by those skilled in the art.

50 As will be apparent to those skilled in the art, it is customary to employ substantially the following procedure in modern paper making practice: Fibrous materials together with filler, size, such as rosin size, size precipitant, such as alum, and coloring matter if desired, are ordinarily mixed in a beater or the like at a dry solid content of approximately 5 per cent. or slightly higher, and are subjected to a beating treatment in the beater, 55 the amount of such treatment depending upon the type of paper which is to be made. The paper mix is then ordinarily discharged from the beater and introduced into a container commonly called a "beater chest", addition- 60 al water usually being added. Thereafter the mix is pumped from the beater chest to a suitable refining engine, usually a Jordan, at a dry solid content of approximately 4 per cent. In common practice the mix is usually diluted somewhat by the addition of water, 65 and the diluted mix is ordinarily conducted from the Jordan to another container commonly known as a "machine chest". From the machine chest the mix is pumped to a point near the web-forming end of the paper machine where it is largely diluted with water, water being added ordinarily in such an amount as to provide a dry content of from approximately  $\frac{1}{2}$  of 1 per cent. or slightly 70 higher, but practically never in excess of  $\frac{1}{2}$  per cent. The mix in such highly dilute condition is then passed through rifflers or the like if desired and thereafter through screens and through the head box of the paper machine onto the machine wire or into the 75 vat depending upon whether a Fourdrinier or a cylinder machine is employed, and during this passage additional amounts of water are usually added in the form of sprays or otherwise. This exact procedure is not always followed but in some instances is modified 80 in accordance with the type of paper being made. For example, in the manufacture of certain types of paper, the beating process is almost or entirely dispensed with, the ingredients of the stock being merely mixed prior to jordaning. In some instances the step of refining or jordaning may be partially or wholly dispensed with. Moreover, 85 the arrangement of the chests in respect to the mechanical treating apparatus is not in all cases precisely as described above.

90 The time consumed from the point of mixing the ingredients in relatively concentrated state up to the point where the stock is to be diluted for delivery to the web-forming end of the machine is relatively long in comparison with the time during which the stock exists in dilute condition prior to its delivery to the web-forming end of the 95 paper machine. The length of time during which the mix remains in a relatively concentrated condition may vary, of course, according to conditions, but it may be anywhere from as little as 15 or more minutes, 100 as in certain extreme cases, up to a matter of a number of hours. On the other hand, the time during which the mix exists in a dilute stage prior to its delivery to the web-forming end of the machine is in some cases a 105 matter of only a few seconds and ordinarily not over a minute. Even under extreme conditions the time would never be in excess of 110 5 minutes.

115 In many instances the water supplied to the beater and also the water employed for dilution at the Jordan as well as for the final dilution of the mix before delivering to the web-forming end of the paper machine consists in whole or in part of "white water" 120 125 130

by which term is meant to be included all effluents from the web-forming end of the paper machine. It will be apparent therefore that this water functions cyclically in the process and that there may be reintroduced into the earlier stages of the process part of the material which was derived from the web-forming stage of the process, such material being returned through the medium of the "white water".

Moreover in modern paper making practice there is a tendency to reclaim the ingredients contained in the white water, sometimes merely from that portion of it which is in excess of that which can be or is to be used cyclically in the process, or sometimes from a portion or from all of that which is to be used cyclically, or both, by subjecting the white water to some suitable procedure, as filtration, such for instance as "deckering" or actual passage through a filtering machine, or sedimentation or the like, thereby passing out the substantially purified aqueous effluent to waste, or for further use in the pulp or paper making process, with the simultaneous return of the recovered material to the paper making process. In some installations this recovered material may be returned to the beater, while in others it may be returned to the beater chest, machine chest, or other point in the process if desired.

It will therefore be apparent that independent of the exact type of apparatus and procedure employed, the following operations are normally employed in the paper making process; the mixing of the ingredients in relatively concentrated form; their contact in such concentrated form for a relatively long period of time; their subsequent dilution to a concentration suitable for delivery to the web-forming end of the paper machine; their remaining in such dilute condition a relatively short period of time; and the recontacting of the mixture of the ingredients prior to its delivery to the web-forming end of the paper machine with the cyclically returned white water and/or material recovered therefrom.

I have found as stated above that a mix made from fibrous materials, sodium resinate, a substantially nonbreakable paraffin emulsion, alum, and carbonate filler, gradually has its sizing deteriorated by the carbonate filler, the degree of deterioration varying with the time of contact and intimacy of contact of the carbonate filler with the rest of the mix.

I have also discovered, as stated above, that such a mix will have its sizing effect restored, thus producing a satisfactorily sized paper, if certain suitable materials are added to the mix later in the paper making operation, at or subsequent to the point where the mix is largely diluted as described above prior to its delivery to the web-forming end

of the paper machine. Thus the material constituting the sizing, the effect of which has been deteriorated or destroyed, acts as a potential sizing agent which is made effective through the addition of a restoring agent.

I have also discovered that this restoring action is relatively sensitive and of relatively brief duration and if the attempt is made to effect the restoration in the mix when it is relatively concentrated, and particularly when the relatively concentrated mix is subjected to agitation as is normal in the stock chests in paper making, that the restorative action is again destroyed. However, I have further discovered, if after applying the restorative action the mix is subjected to a minimum degree of intimate contact and a minimum of time of contact, such as is the case when the mix is in dilute form prior to its delivery to the web-forming end of the paper machine, then the restorative action is practically not affected or only slightly affected according as the intimacy and/or time of contact may be lesser or greater. Also I have found that agitation in the dilute state has a very much less injurious effect than in the concentrated.

I have found in general that acidic material and/or salts of trivalent metals, such as ferric iron or aluminum, act as restorative agents. For example, I have found that it is possible to restore the sizing effects to a mix containing carbonate filler in which the sizing effect has been destroyed, by addition of an acid such as sulphuric acid ( $H_2SO_4$ ). I have also found it possible to use acid salts such as sodium bisulphate ( $NaHSO_4$ ). However, the best agents I have so far found are the salts of the trivalent metals, such as ferric iron or aluminum, and of these aluminum has by my tests to date proven to be the better. Ferric iron may be used in papers other than white, but for white papers, of course, aluminum is the most suitable material, and even for colored papers, its relative greater effectiveness may render it more economical.

Of the aluminum salts available the chloride, sulphate, or the like, or the double salts which are the true alums, may be used, but because of economy, the ordinary sulphate of aluminum normally known as "alum" is most suitable. I have found that any of the ordinary types of alum are satisfactory, whether acid, neutral, or basic. I have also found that whereas the acidic materials mentioned in the preceding paragraph can be used and although some of them are considerably cheaper than alum, that the effectiveness of alum seems to be sufficiently greater in proportion to the above mentioned materials, that it becomes economical to use alum instead of these relatively cheaper materials.

Therefore the method I prefer to employ

to restore the sizing consists substantially of adding a subsequent portion of alum, preferably continuously, in the paper making process as near as feasible to the point of web formation on the paper machine, preferably at or following the point at which the paper mix is largely diluted as indicated above.

The emulsions which I have found to be substantially unaffected by ordinary materials in the concentration at which they exist in the paper making process may be made in a variety of ways, for instance, with gums such as gum ghatti or gum arabic. While dextrin of itself does not appear to be suitable as an emulsifying agent, particularly if the emulsion is to be stored for any appreciable time, it does however appear to be useful in connection with the gums mentioned above. As the gums are normally much more expensive than dextrin, the dextrin may thus be used in conjunction with the gums to produce in general a lower cost emulsion. I have tested several formulæ involving the use of gums and dextrin which give emulsions of essentially the nature desired, and which appear to work satisfactorily for the purpose. However, the one which I prefer to use in practice and which I have found to work well on a practical scale, is an emulsion made of paraffin with gum ghatti and dextrin as emulsifying agents. In one such emulsion, for example, which proved satisfactory, I used by weight as follows:

15 parts paraffin, 1 part gum ghatti, 1 part dextrin, 83 parts water.

As stated above so far as I have been able to discover by experiment, the emulsions which I employ are not affected in any way by any of the chemicals with which they come in contact at the concentrations at which they are used in the paper making process, nor are they affected by any of the mechanical agencies with which they come in contact at the intensities at which they are normally employed in the paper making process.

The reason for this latter characteristic is probably that the particles in my emulsions are surrounded with a film as set forth previously which is one or more molecules in thickness and hence entirely of negligible thickness compared with any solid particle film. Hence such films cannot be knocked off or ruptured by ordinary mechanical means, as the thickness of this film is of entirely different order of magnitude (smaller) than are the clearances which obtain in the paper making machinery. This of course is not the case with emulsifiers of the insoluble type which possess much thicker films, whether the films so produced be made up of individual particles of materials like clay, or whether they be of jelly-like character such as is the case where certain insoluble materials are employed which are of that character, whether introduced as one material or producer in situ

by the reaction of the two or more materials.

Of course it is not necessary that the emulsifier I use be water soluble in the sense that sodium chloride, for instance, is soluble, as materials which are known in the art as being colloidally soluble, are also suitable. For example gum ghatti which is suitable for my use may be considered to be in a measure colloidally soluble. With emulsifiers of the type I employ the condition of the layer surrounding the disperse phase is such that by mechanical action in the paper making process, this layer is not disrupted, and therefore, the emulsion remains substantially non-breakable as heretofore indicated.

It is to be understood that I do not confine myself to the materials indicated above as being suitable for my emulsion since now that the principle of the use of a substantially non-breakable paraffin emulsion which is capable of having its disperse phase concentrated has been established in the paper industry, doubtless other similar emulsions will be evolved. Nor do I confine myself to the definite concentration of the paraffin in the emulsion nor to definite proportions of emulsifying agents to each other or to the paraffin, as these may be varied in considerable degree without affecting the desirable qualities of the emulsion.

Emulsions of the character referred to may be made in a variety of ways, as for example, in a dispersion machine such as any of a number of colloid mills or homogenizers. A suitable way is to melt the paraffin, dissolve the emulsifying agent or agents in water, heat the emulsifying agent solution above the melting point of the paraffin and then feed the melted paraffin and the heated solution of emulsifying agents jointly to the emulsifying machine.

In regard to the paraffin used, it is to be understood that either low or high melting point material can be employed. The so-called fully refined paraffin is entirely satisfactory since it does not impart objectionable color to white sheets. However, for purposes of economy, it is often desirable to use a less pure material such for example as the material which is commonly known to the trade as semi-refined paraffin scale, containing approximately  $\frac{1}{2}$  per cent. of oil and water as impurities, which material gives satisfactory results. Such material will perhaps in certain cases have varying melting points, but one particular sample used, for example, had a melting point of approximately  $115^{\circ}$  F. ( $46^{\circ}$  C.). Other even more impure paraffins may be used, especially if the color (whiteness) requirements of the finished paper are not too exacting, or if papers, other than white, are to be made.

In the preferred practice of my invention I add to the beater or other similar or mixing or compounding or disintegrating or treating machine all the pulp or other fibrous ma-

terials to be employed except those coming under the definition of carbonate filler herein-after set forth, and such fibrous material as is in the stock of the recovered white water. 5 Thereafter I add sodium resinate, a substantially nonbreakable paraffin emulsion preferably in dilute form, and incorporate them thoroughly with the pulp. Alum is then added. After the sodium resinate-alum concentrating precipitate has been formed on the fibre I then add if desired fibrous materials coming under the definition of carbonate filler herein-after set forth and/or carbonate filler itself. It is possible to add all the fibrous 10 constituents and/or the carbonate filler itself in the beater prior to the addition of the alum but my experiments have indicated that better results are obtainable when the sodium resinate alum concentrating precipitate is 15 formed on the fibre in the absence of any carbonate filler.

Moreover in furnishing the beater, I preferably use fresh water or white water which has been clarified so that the sodium resinate 20 alum precipitate may be completely formed on the fibre before the addition of carbonate filler in any form to the mix.

In regard to the mixing of the ingredients of fibre (free from carbonate filler), and the 25 other ingredients as indicated above, I do not confine myself strictly to the order of addition indicated above, but I have found that a suitable way is to allow sufficient time for the sodium resinate and the substantially non-breakable paraffin emulsion to be thoroughly 30 incorporated with the fibre prior to the addition of the alum.

Furthermore, fillers of types other than 35 carbonate fillers may be also added in the beater if it be desired to employ them in conjunction with the carbonate fillers in the paper, as well as coloring materials, and other substances which may normally be added in the paper making process.

40 In this connection, with the use of the carbonate filler, starch may be added, if desired, to the mix in the beater or other point in the process, attention being directed to my copending application Serial No. 202,453, filed 45 June 29, 1927. The mix in the beater may then be given the usual treatment, passed through the beater chest, Jordan and machine chest. All waters used subsequent to the precipitation of the sodium resinate alum 50 55 concentrating precipitate in the beater may be either fresh water or white water, as desired.

The mix still in relatively concentrated 60 form is now at the point where it is ready for dilution preparatory to delivery to the web-forming end of the paper machine. Here the white water from the paper machine may be used as diluting water. At this point or subsequent thereto, alum is added preferably 65 continuously, preferably in solution, the pre-

caution being taken that adequate mixing of the alum, the white water and other water if used, and the relatively concentrated mix coming from the machine chest is insured. A separate mixing box may be provided if desired but under ordinary machine practice this is unnecessary since there is usually adequate provision made in paper manufacturing to insure thorough mixing of the relatively concentrated mix with the diluting water. I have found in practice that it is also satisfactory to add the alum at a point subsequent to this, for example, just prior to the passage of the diluted mix to the screens, the screens affecting very thorough mixing in this case. If, however, the alum is actually added at the head-box of the machine subsequent to the screens, care should be taken that adequate distribution and mixing of the ingredients is insured by proper baffling or the like.

An illustrative furnish which may advantageously be used in practicing my invention is as follows:

#### Materials added in the beater

|                                                                              | Pounds |
|------------------------------------------------------------------------------|--------|
| Fibrous furnish (e. g. sulphite and soda pulps)                              | 1700   |
| Rosin (added in the form of sodium resinate)                                 | 10     |
| Paraffin (added in the form of substantially nonbreakable paraffin emulsion) | 30     |
| Alum (ordinary $Al_2(SO_4)_3 \cdot 18H_2O$ )                                 | 30     |
| Calcium carbonate magnesium hydroxide (carbonate filler)                     | 300 95 |

#### Material added proportionately and continuously on dilution

|                                                                     | Pounds |
|---------------------------------------------------------------------|--------|
| Restoring agent, e. g. alum (ordinary $Al_2(SO_4)_3 \cdot 18H_2O$ ) | 50     |

Another illustrative furnish is as follows:

#### Materials added in the beater

|                                                                                          | Pounds  |
|------------------------------------------------------------------------------------------|---------|
| Fibrous furnish (e. g. approximately equal parts of sulphite, soda and old paper stocks) | 1530    |
| Rosin (added in the form of sodium resinate)                                             | 10 105  |
| Paraffin (added in the form of substantially nonbreakable paraffin emulsion)             | 30      |
| Alum (ordinary $Al_2(SO_4)_3 \cdot 18H_2O$ )                                             | 30      |
| "Broke" (containing calcium carbonate magnesium hydroxide (carbonate filler))            | 170     |
| Calcium carbonate magnesium hydroxide (carbonate filler)                                 | 300 110 |

#### Material added proportionately and continuously on dilution

|                                                                     | Pounds |
|---------------------------------------------------------------------|--------|
| Restoring agent, e. g. alum (ordinary $Al_2(SO_4)_3 \cdot 18H_2O$ ) | 50     |

In the above formulæ, the weights of carbonate filler refer to the bone dry basis, the weights of all other ingredients being given on the air dry basis.

In either of the above furnishes starch may be used. It may be conveniently added to the beater subsequent to the addition of the carbonate filler, or otherwise if desired. Suitable coloring matter may be added if desired.

The illustrative furnishes given above produce satisfactorily sized paper, and, as will be apparent, the sizing can be increased or decreased by varying the relative quantities of the materials used in the above formulæ. The resultant paper may be used for 130

such purposes as those to which sized papers are normally put including that as a raw stock for further conversion as for example for coating.

5 While I have described herein the effect of sodium resinate and alum as mutually precipitating agents to produce a concentrating effect on the disperse phase of a substantially nonbreakable paraffin emulsion, other materials may be used, as for instance, soaps other than sodium resinate, or any partially or completely saponified material, such as saponified beeswax. Moreover, in place of alum as one of the mutually precipitating 10 agents and as a sizing restoring agent of the character referred to, I may employ salts of other trivalent metals, such as ferric iron. Also, I may employ in place of ordinary alum other salts of aluminum, such as the 15 chloride, or the like. In addition, sodium bisulphate may be employed with a certain measure of success.

When I employ the term "paraffin" herein, I mean paraffin wax, which is solid at 20 ordinary or room temperature. I do not mean to restrict myself only to the paraffin hydrocarbons, but mean to include in this term all the hydrocarbons of a waxy nature substantially unsaponifiable and inert to 25 acidic and alkaline materials under ordinary conditions of temperature and pressure, whether derived from petroleum, shale, lignite, earth wax, or other natural or artificial sources. I do not, however, mean to include 30 in this term material of a pitchy nature, such as bitumen or asphalt.

By the term "carbonate filler" as employed 35 herein is meant the substantially water insoluble normal or basic carbonates of alkaline earth metals (which expression is herein intended to include magnesium), or compounds, or double salts, or physically associated mixtures of these with one or more other acid soluble materials of a substantially 40 water insoluble nature, these fillers whether simple or complex as above, being characterized by the fact that, when agitated in contact with freshly boiled distilled water in concentrated suspension for 45 say an hour, they impart to the water a pH value which is on the alkaline side of the neutral point, and also by the fact that they give off carbon dioxide gas when brought into contact with an aqueous mineral acid, e. g. 50 hydrochloric acid. Examples of such fillers are calcium carbonate, of which lime mud from the causticizing process is one form; calcium carbonate magnesium basic carbonate 55 employed in the paper disclosed in my U. S. Patent No. 1,595,416 of August 10, 1926; and calcium carbonate magnesium hydroxide disclosed in my U. S. Patent No. 1,415,391 of May 9, 1922. As will be apparent, these fillers are referred to not only 60 in their chemically pure form but also in

commercial form containing such impurities as may occur in such commercial products; and also when present with other material, so that they constitute only a part, either major or minor, of the whole. It should be 70 stated that any given filler of the type referred to is not necessarily of uniform particle size; nor are the average particles sizes of the fillers necessarily alike, as some of the fillers of the type referred to have relatively 75 coarse grain particles, whereas others are much more finely divided, and some are so finely divided that they may be said to approach or be in the colloidal condition.

Moreover, by the term "carbonate filler", 80 I mean to include not only the case where the carbonate filler is added as such in the paper making process, but also the case where it may be added wholly or in part incorporated with fibrous material and/or other material such as paper coating constituents or the like. Such a case would be where paper made with carbonate filler, either as a filling or coating constituent, or both is reused in the paper making process. Such papers may 85 be those known to the trade as "old papers" or "old waste papers" or "waste papers" in any form, or returned trimmings or damaged paper or the like, or they may be the "broke", that is, the partially made, the imperfect, or 90 the waste paper which accompanies the paper making, finishing, storing, packing, shipping, or the like operations in a paper mill, and which is reworked either in the same or some other mill. Such papers are 95 sometimes reworked by themselves and added in broken down or in pulp form in the paper making process, being treated or cooked in some cases with or without chemicals and washed if desired, this reworking meaning 100 to include the process of deinking if such is practiced or of bleaching or of both deinking and bleaching, or sometimes they are added directly in the paper making process and broken down to pulp form therein. In 105 any event they are a source of carbonate filler in the paper to be made, and are included in the term "carbonate filler" as used herein.

When I use the word "paper" herein, I 110 use it in the broad sense to include products of manufacture of all types and of all weights and thicknesses, which contain as an essential constituent a considerable amount of prepared fibre and which are capable of being produced on a Fourdrinier, cylinder, or other forming, felting, shaping or molding machine.

115 Although the expression "wet end of the paper machine" may at times be used to convey various meanings, where I use the expression in the claims I intend it to include those instrumentalities provided in paper manufacture by which and/or in which the relatively concentrated mix is diluted, and 120 treated, conveyed or fed up to the point of 125 130

web formation, such as the mixing box, regulating and proportioning devices, riffles, troughs, screens, machine head boxes, inlets, and the like, including also instrumentalities used in the white water cycle, but I do not intend to include in this definition the web-forming device itself, that is, the moving wire in the case of a Fourdrinier machine or the cylinder mold in the case of a cylinder machine.

10 Although I have described in detail several illustrative furnishes I do not intend to be limited thereby, as my invention may be practiced with a broad variety of formulæ, 15 using various materials customarily employed for various grades of paper in any suitable proportions. Moreover, various changes in procedure, ingredients, and arrangement of steps may be resorted to in the 20 practice of my invention without departing from the spirit of my invention or the scope of the subjoined claims.

I claim:

1. The method of manufacturing a sized 25 paper filled with carbonate filler comprising adding to fibrous material a substantially nonbreakable paraffin emulsion and a substance which will react with a second substance subsequently added to form a precipitate, adding said second substance, the reaction caused thereby serving to concentrate the disperse phase of said paraffin emulsion but not to break said emulsion, adding carbonate filler, thereafter adding a sizing 30 restoring agent under conditions favoring the minimizing of the time of contact of the constituents of the mix, and thereafter making paper therefrom.

2. In a method of manufacturing a sized 40 paper filled with carbonate filler, the step of adding to a paper mix containing carbonate filler which paper mix has been previously sized by concentrating thereon the disperse phase of a substantially nonbreakable paraffin emulsion by the precipitation of two mutually reacting substances, a sizing restoring agent under conditions favoring the minimizing of the time of contact of the constituents of the mix.

3. The method of manufacturing a sized 50 paper filled with carbonate filler comprising adding to fibrous material a substantially nonbreakable paraffin emulsion and a substance capable of reacting with a second substance subsequently added to form a precipitate upon the fibrous material, adding said second substance, the reaction caused thereby serving to concentrate in association with said precipitate the disperse phase of said 55 paraffin emulsion but not to break said emulsion, said precipitate being substantially incapable of having the paraffin associated therewith released from emulsified condition by mechanical means, adding carbonate filler, thereafter adding a sizing restoring agent

under conditions favoring the minimizing of the time of contact of the constituents of the mix, and thereafter making paper therefrom.

4. The method of manufacturing a sized 60 paper filled with carbonate filler comprising adding to fibrous material a substantially nonbreakable paraffin emulsion and a substance which will react with a second substance subsequently added to form a precipitate, adding said second substance, the reaction caused thereby serving to concentrate the disperse phase of said paraffin emulsion but not to break said emulsion, adding carbonate filler, thereafter adding a salt of a trivalent metal under conditions favoring 65 the minimizing of the time of contact of the constituents of the mix, and thereafter making paper therefrom.

5. The method of manufacturing a sized 70 paper filled with carbonate filler comprising adding to fibrous material a substantially nonbreakable paraffin emulsion and a substance which will react with a second substance subsequently added to form a precipitate, adding said second substance, the reaction caused thereby serving to concentrate the disperse phase of said paraffin emulsion but not to break said emulsion, adding carbonate filler, thereafter adding a salt of aluminum under 75 conditions favoring the minimizing of the time of contact of the constituents of the mix, and thereafter making paper therefrom.

6. The method of manufacturing a sized 80 paper filled with carbonate filler comprising adding to fibrous material a substantially nonbreakable paraffin emulsion and a substance which will react with a second substance subsequently added to form a precipitate, adding said second substance, the reaction caused thereby serving to concentrate the disperse phase of said paraffin emulsion but not to break said emulsion, adding carbonate filler, thereafter adding a salt of aluminum under 85 conditions favoring the minimizing of the time of contact of the constituents of the mix, and thereafter making paper therefrom.

7. The method of manufacturing a sized 90 paper filled with carbonate filler comprising adding to fibrous material a substantially nonbreakable paraffin emulsion and a substance which will react with a second substance subsequently added to form a precipitate, adding said second substance, the reaction caused thereby serving to concentrate the disperse phase of said paraffin emulsion but not to break said emulsion, adding carbonate filler, thereafter adding a sizing restoring agent at a point in the process subsequent to that at which the paper mix exists 95 in relatively concentrated form, and thereafter making paper therefrom.

8. In a method of manufacturing a sized 100 paper filled with carbonate filler, the step of adding to a paper mix containing car-

- bonate filler, which paper mix has been previously sized by concentrating thereon the disperse phase of a substantially nonbreakable paraffin emulsion by the precipitation of two 5 mutually reacting substances, a salt of a trivalent metal under conditions favoring the minimizing of the time of contact of the constituents of the mix.
9. In a method of manufacturing a sized 10 paper filled with carbonate filler, the step of adding to a paper mix containing carbonate filler, which paper mix has been previously sized by concentrating thereon the disperse phase of a substantially nonbreakable paraffin emulsion by the precipitation of two 15 mutually reacting substances, alum under conditions favoring the minimizing of the time and intimacy of contact of the constituents of the mix.
10. The method of treating a paper mix originally containing carbonate filler and fibrous material having incorporated therewith the disperse phase of a substantially nonbreakable paraffin emulsion in association 20 with the precipitate produced by two mutually reacting substances, comprising adding to such mix a salt of a trivalent metal at the wet end of the paper machine.
11. The method of treating a paper mix 25 originally containing carbonate filler and fibrous material having incorporated therewith the disperse phase of a substantially nonbreakable paraffin emulsion in association with the precipitate produced by two 30 mutually reacting substances, comprising adding to such mix alum at the wet end of the paper machine.
12. The method of manufacturing a sized 35 paper filled with carbonate filler comprising mixing with fibrous material a substantially nonbreakable paraffin emulsion, saponified material, a precipitant therefor, and carbonate filler, thereafter adding a sizing restoring agent under conditions favoring the 40 minimizing of the time of contact of the constituents of the mix, and thereafter passing the mix on to a web-forming device.
13. The method of manufacturing a sized 45 paper filled with carbonate filler comprising mixing with fibrous material a substantially nonbreakable paraffin emulsion, saponified material, a precipitant therefor, and carbonate filler, thereafter adding a sizing restoring agent at the wet end of the paper machine, and thereafter making paper therefrom.
14. The method of manufacturing a sized 50 paper filled with carbonate filler comprising mixing with fibrous material a substantially nonbreakable paraffin emulsion, saponified material, a precipitant therefor, and carbonate filler, thereafter adding alum at the wet end of the paper machine, and thereafter making paper therefrom.
15. The method of manufacturing a sized 55 paper filled with carbonate filler comprising mixing with fibrous material a substantially nonbreakable paraffin emulsion, soap, a precipitant therefor, and carbonate filler, thereafter adding alum at the wet end of the paper machine, and thereafter making paper therefrom.
16. The method of manufacturing a sized 60 paper filled with carbonate filler comprising mixing with fibrous material a substantially nonbreakable paraffin emulsion, sodium resinate, a precipitant therefor, and carbonate filler, thereafter adding alum at the wet end of the paper machine, and thereafter making paper therefrom.
17. The method of manufacturing a sized 65 paper filled with carbonate filler comprising mixing with fibrous material a substantially nonbreakable paraffin emulsion, sodium resinate, alum, and carbonate filler, thereafter adding alum at the wet end of the paper machine, and thereafter making paper therefrom.
18. The method of manufacturing a sized 70 paper filled with carbonate filler comprising mixing with fibrous material a substantially nonbreakable paraffin emulsion, sodium resinate in an amount insufficient of itself to impart a substantial degree of sizing to the paper, alum, and carbonate filler, thereafter adding alum at the wet end of the paper machine, and thereafter making paper therefrom.
19. The method of manufacturing a sized 75 paper filled with carbonate filler comprising mixing with fibrous material a paraffin emulsion made with gum ghatti as emulsifying agent, sodium resinate, alum, and carbonate filler, thereafter adding alum at the wet end of the paper machine, and thereafter making paper therefrom.
20. The method of manufacturing a sized 80 paper filled with carbonate filler comprising mixing with fibrous material a substantially nonbreakable paraffin emulsion made with gum ghatti and dextrin as emulsifying agents, sodium resinate, alum and carbonate filler, thereafter adding alum at the wet end of the paper machine, and thereafter making paper therefrom.
21. A sized paper comprising fibrous material, carbonate filler, the reaction product of sodium resinate and alum, said sodium resinate having been originally present in an amount insufficient of itself to impart a substantial degree of sizing to the paper, and paraffin.
- In testimony whereof I affix my signature.  
HAROLD ROBERT RAFTON.
- 125
- 130